

# UNITED STATES PATENT OFFICE.

JOSEPH DE COSMO AND HENRI QUINAUX, OF LIEGE, BELGIUM.

## FUEL FOR INTERNAL-COMBUSTION ENGINES.

1,184,727.

Specification of Letters Patent.

Patented May 30, 1916.

No Drawing.

Application filed May 15, 1913. Serial No. 767,878.

*To all whom it may concern:*

Be it known that we, JOSEPH DE COSMO and HENRI QUINAUX, both subjects of the King of Belgium, and residing at 20 Rue de 5 la Vieille Montague and 37 Rue Dony, in Liege, Belgium, have invented certain new and useful Improvements in Fuel for Internal-Combustion Engines; and we do hereby declare the following to be a full, clear, and 10 exact description of the invention, such as will enable others skilled in the art to which it appertains to make and use the same.

The present invention relates to a new and economical fuel for explosion motors 15 of all descriptions, produced by mixing different substances in suitable proportions.

It is well known that the price of petrol, which is at present generally used for running motors, tends to rise continually and 20 endeavors are being made to find less costly fuels. With that object in view the heavy oils have been tried, but there are various difficulties in using them in the engines of motor cars, such as incomplete combustion, 25 the necessity of heating the carburetor, which causes deposits of carbon that clog up the orifices and the sparking plugs, and so on. It has also been proposed to utilize crude naphthalene or white naphthalene, 30 but as naphthalene will not liquefy or retain the liquid condition at a lower temperature than about 80° C., it has been found necessary to use special carburetors.

The essential feature of the present invention is the solution in refined mineral oil of a substantial proportion of naphthalene, which by the aid of suitable additional substances is maintained in solution at ordinary temperatures in a condition in which the 40 mixture is readily vaporized. The additional substances by which we effect solution of the naphthalene are nitro-naphthalene, naphthylamin and cresol, in proportions which may vary with the nature of the 45 oil and the amount of naphthalene to be

dissolved. The following proportions and method of mixing have been found suitable:—

|                     |     |        |    |
|---------------------|-----|--------|----|
| Crude naphthalene   | 400 | grams. | 50 |
| Refined mineral oil | 600 | "      |    |
| Nitro-naphthalene   | 10  | "      |    |
| Naphthylamin        | 5   | "      |    |
| Cresol              | 5   | "      |    |

These substances are mixed together preferably as follows: The crude naphthalene is first mixed with half the quantity of mineral oil (300 grams), then the nitro-naphthalene and the naphthylamin are added, and the mixture is brought to a temperature of from 23 to 30° cent., according to the quality of the naphthalene used. The mixture maintains its liquid state at these and even at lower temperatures. Finally, the rest of the mineral oil is added, and the whole strongly agitated by means of a rotating central stirrer or any other convenient contrivance. When in consequence of the centrifugal action, the liquid has formed a central depression the cresol is poured in, which homogenizes the mixture. The liquid fuel is then decanted, allowed to rest for ten or twelve hours to permit any impurities to settle, and is then filtered off.

The nitronaphthalene and naphthylamin may be used singly, as they have substantially the same effect but usually a mixture would be employed, the relative proportions of which may depend on the cost of each of these substances. The proportions of all the ingredients may vary according to the nature of the mineral oil employed and according to other circumstances, the above figures and method being given merely by way of example. The best results are generally obtained by using mineral oil of about 0.760 or lower specific gravity. The function of the nitro-naphthalene and naphthylamin is to liquefy the naphthalene while the cresol converts the whole into a

homogeneous mixture, which is cheap and efficient, is free from acidity and has much the same viscosity as petrol.

Having thus described our invention, we 5 claim:—

1. A liquid fuel for explosion engines containing a substantial proportion of naphthalene, mineral oil, and naphthyllic compound, and cresol.
- 10 2. A liquid fuel for explosion engines containing a substantial proportion of naphthalene, mineral oil, naphthylamin, and cresol.

3. A liquid fuel for explosion engines containing a substantial proportion of 15 naphthalene, mineral oil, naphthylamin, nitro-naphthalene, and cresol.

In testimony that we claim the foregoing as our invention, we have signed our names in presence of two subscribing witnesses.

J. DE COSMO.  
H. QUINAUX.

Witnesses:

L. R. DELLICOUR,  
A. PENDLETON CRUGER.